

1

3,403,013

**METHOD OF OPERATING AN INTERNAL COMBUSTION ENGINE AND MOTOR FUEL THEREFOR**

George W. Eckert, Wappingers Falls, N.Y., assignor to Texaco Inc., New York, N.Y., a corporation of Delaware

No Drawing. Filed Apr. 11, 1967, Ser. No. 629,897  
12 Claims. (Cl. 44—71)

**ABSTRACT OF THE DISCLOSURE**

There is disclosed a method for operating an internal combustion gasoline engine and a novel motor fuel composition for said process comprising a mixture of hydrocarbons in the gasoline boiling range and a substituted urea.

The present invention relates to a method for operating an internal combustion engine which gives a substantial improvement in fuel economy. This invention also relates to a novel fuel composition for use in the process comprising a mixture of hydrocarbons in the gasoline boiling range containing a viscosity thickening amount of an oil-soluble substituted urea.

Methods for improving fuel economy in the operation of gasoline-powered automobiles by altering the physical properties of the fuel have been described before. For example, the viscosity of gasoline can be increased so that effective engine operation is obtained using leaner fuel-air ratios under normal driving conditions. Not only is the fuel consumption of the gasoline-burning automobile substantially reduced but the improvement is realized without any mechanical change in the carburetor or other parts of the engine. Such a method is disclosed in U.S. Patent 3,164,138 which issued on Jan. 5, 1965.

The present invention is based on the discovery that substituted ureas are effective for modifying the fluid properties of gasoline. More specifically, an economical engine operation is achieved by burning a gasoline in which the viscosity has been substantially increased due to the addition of a substituted urea to the fuel composition. The viscosity increase in the gasoline gives a lower rate of gasoline flow through the carburetor under ordinary level road driving conditions without appreciably altering the specific volume of air entering the engine, thereby producing a leaner fuel-air combustion mixture. Besides improving fuel efficiency the leaner mixture operation results in a reduction of undesirable exhaust emissions from the vehicle.

In accordance with the method of this invention, a spark-ignited internal combustion engine is operated by burning a motor fuel composition containing a viscosity modifying oil-soluble substituted urea formed from the reaction of a specific type of amine with toluene diisocyanate. The motor fuel of the invention comprises a mixture of hydrocarbons in the gasoline boiling range containing an amount of the substituted urea effective to substantially increase the viscosity of the motor fuel over the viscosity of the hydrocarbon mixture. More particularly, the amount of the oil-soluble substituted urea employed in the motor fuel is effective to increase the viscosity of the motor fuel by at least 10% and up to about 200% over the viscosity of the hydrocarbon mixture under the conditions selected for the viscosity determinations. The viscosity of the fuel can be measured by any of the standard methods for viscosity determinations of liquids provided that conditions are selected to minimize discrepancies which could arise from the evaporation of highly volatile components of the gaso-

2

line. The viscosity of the gasolines described herein was measured by the Kinematic Viscosity Procedure (units in centistokes) at 77° F.

The oil-soluble substituted ureas which have been found effective for thickening the fuels of the invention are represented by the following formula:



in which R and R' are each alkyl radicals having from 1 to 18 carbon atoms and the sum of the carbon atoms in all the R and R' radicals is at least 12 and preferably at least 18. The foregoing compounds are prepared by reacting a secondary alkyl primary amine with a toluene diisocyanate having the formula:



Two moles of amine are reacted with one mole of diisocyanate to produce the effective substituted urea for the motor fuel of this invention. It will be appreciated that toluene diisocyanate is a commercial product consisting of a mixture of isomeric toluene diisocyanates.

The amines which can be reacted with toluene diisocyanate to produce the viscosity increasing urea additive of this invention are secondary alkyl primary amines, i.e. monoamines, in which the amino group is attached to a secondary carbon atom. These amines correspond to the formula:



in which R and R' are alkyl radicals having from 1 to 18 carbon atoms with the sum of the carbon atoms in R and R' being at least 6. Secondary alkyl primary amines are commercially available generally as mixtures of amines having alkyl radicals in a narrow molecular weight range. An n-alkyl primary beta amine having an average molecular weight of about 170 and an average of about 11 carbon atoms is marketed as Armeen L-9. Armeen L-11 is an n-alkyl primary beta amine having an average molecular weight of 205 and an average of 13 carbon atoms. These are described on page 40 of "Chemical Engineering News," dated Jan. 11, 1965. Other effective secondary alkyl primary amines are 2-amino octane, 3-amino octane, 4-amino octane, 3-amino decane and 2-amino dodecane. The preferred amines are those in which the sum of the carbon atoms in R and R' is at least 9.

The nature of the amine component of the substituted urea is critical to the process and motor fuel of this invention. Many amines which react with toluene diisocyanate to form substituted ureas are insoluble in or otherwise ineffective for increasing the viscosity of gasoline. These amines are clearly outside of the scope of the present invention. Examples of amines which do not form effective substituted ureas when reacted with toluene diisocyanate include monoamines, such as aniline, benzylamines, cyclohexylamine, ethoxyethylamine, stearylamine and p-toluidine and diamines, such as N-2-undecyl-1,3-propane diamine.

It is essential that the oil-soluble substituted urea of the invention substantially increase the viscosity of the motor fuel composition over the viscosity of the hydrocarbon

mixture or base fuel. A viscosity increase of at least 10% in the motor fuel measured as the kinematic viscosity in centistokes is critical to provide a distinct improvement in fuel economy. This determination may be made at any convenient temperature, such as at 77° F. in the present invention, or at 0° F. as in the above-noted patent. Actually, the viscosity of a gasoline can be increased by several hundred percent or more by adding an oil-soluble viscosity modifying substituted urea. However, a viscosity increase in the range of at least 10 to about 200% is the critical range to produce the desired operating economies. Viscosity increases from about 20 to 100% are preferred with optimum results being realized with viscosity increases of from 40 to 100%. The foregoing viscosity increases are generally realized by employing the oil-soluble substituted urea of the invention in an amount from about 0.005 to 0.5 weight percent based on said gasoline. Preferred amounts of the substituted urea in gasoline range from about 0.01 to 0.2 weight percent. Excessively high viscosity increases, that is, a viscosity increase substantially over 300% generally, produce a fuel having unsatisfactory flow properties. Such viscosity increases in a fuel sufficient to reduce the fuel/air ratio to less than 0.06 will also generally result in misfiring and loss of power.

A base fuel or gasoline without the viscosity modifying oil-soluble substituted urea of the invention will generally have a kinematic viscosity in centistokes at 77° F. in the range of 0.500 to 0.600. Any gasoline of either high or low octane value or high or low volatility can be characterized by its kinematic viscosity in centistokes at 77° F. readily determinable by known methods. An increase in the viscosity of such a gasoline in the order of 10 up to 200%

gine operating at 30 miles per hour under level road conditions showed that the fuel of increased viscosity produced operating economies of 4.5%. Similarly, a premium motor fuel which has had its viscosity increased by 24.6% when tested in a General Motors Research Engine at 30 miles per hour level road conditions showed that the fuel/air ratio was reduced by about 17% and that the fuel economy was improved by about 7.2%.

Gasolines which have had their viscosities increased in the order of 50% according to this invention have shown substantial improvements in fuel economy ranging from 5 to 10% or more over the base fuel depending on the load conditions employed. Similarly, gasolines that have had their viscosity increased in the order of 100% or more have been observed to provide fuel economies substantially in excess of 20%.

The effect of the substituted ureas of this invention was determined in the following test. The base fuel employed was a premium gasoline containing 3.09 cc./gallon of tetraethyl lead fluid mixture. This gasoline had a Research Octane No. of 101.2, a boiling range from 87° F. to 368° F., a kinematic viscosity in centistokes at 77° F. of 0.557 and consisted of 31.5 percent aromatics, 10.5 percent olefins and 58 percent saturates as determined by conventional FIA analysis. The table below gives the concentration of the substituted urea additive in the gasoline in weight percent. Since all of the additives were prepared using toluene diisocyanate only the amine component from which the urea was formed is given in the table. It is understood that the substituted urea additive was prepared by reacting two moles of the amine with one mole of the toluene diisocyanate.

TABLE I—KINEMATIC VISCOSITY OF PREMIUM GASOLINE CONTAINING SUBSTITUTED UREA FORMED BY REACTING TOLUENE DIISOCYANATE WITH THE INDICATED AMINE

| Run | Amine component of substituted urea              | Average mol. wt. of amine | Percent substituted urea in gasoline | Kinematic viscosity, cs. at 77° F. | Increase in viscosity at 77° F., Percent |
|-----|--------------------------------------------------|---------------------------|--------------------------------------|------------------------------------|------------------------------------------|
| 1   | None                                             |                           |                                      | 0.557                              |                                          |
| 2   | n-C <sub>9</sub> alkyl primary beta amine        | 140                       | 0.05                                 | 0.913                              | 64                                       |
| 3   | do                                               | 140                       | 0.10                                 | 0.390                              | 149                                      |
| 4   | n-C <sub>11</sub> alkyl primary beta amine       | 170                       | 0.05                                 | 0.977                              | 75                                       |
| 5   | do                                               | 170                       | 0.10                                 | 1.98                               | 255                                      |
| 6   | C <sub>10-14</sub> secondary alkyl primary amine | 183                       | 0.10                                 | 0.976                              | 72                                       |
| 7   | do                                               | 183                       | 0.20                                 | 1.40                               | 151                                      |
| 8   | 2-ethylhexylamine                                | 120                       | 0.10                                 | 0.681                              | 22                                       |
| 9   | Tertiary C <sub>11-14</sub> alkyl primary amine  | 200                       | 0.05                                 | 0.559                              | 0.3                                      |
| 10  | Tertiary C <sub>18-24</sub> alkyl primary amine  | 300                       | 0.05                                 | 0.560                              | 0.5                                      |

due to the addition of an oil-soluble substituted urea of this invention will produce substantial economies in the operation of a spark-ignited, internal combustion engine.

The motor fuel of this invention can be prepared by admixing a suitable amount of the selected oil-soluble substituted urea directly into the gasoline. Alternatively, the substituted urea can be formed in situ, that is, by adding the components toluene diisocyanate and the amine separately to the gasoline wherein they will react to form a substituted urea corresponding to the formula noted above. It is understood that the motor fuel of the invention can also contain the additives conventionally employed in gasoline, such as alkyllead octane appreciators, alkyl halide lead scavengers, anti-icing additives, corrosion inhibitors, dyes and the like.

As an example of the fuel economies that can be realized by increasing the viscosity of a gasoline, it has been observed that a base motor fuel having a Research Octane Number 99.4 and a kinematic viscosity of 0.928 centistokes at 0° F., which has had its viscosity increased to 1.196 cen-

Runs 2 through 7 illustrate the invention and show a premium gasoline of increased viscosity due to the addition of the specific substituted ureas to produce a fuel providing substantial fuel economies when employed in a car operated under level road conditions. In contrast, the ureas formed using primary alkyl amines as shown in Runs 8 through 10 were essentially ineffective for increasing the viscosity of the gasoline.

Engine tests were conducted in an RDH engine manufactured by Waukesha Motor Company. This 41.4 cubic inch displacement engine had a 9:1 compression ratio. The engine was operated at 1200 r.p.m. or a 30 m.p.h. Level Road Load. The base fuel employed was the premium gasoline described above. The additive containing fuel contained the indicated amounts of the substituted urea formed from the reaction of one mole of toluene diisocyanate and two moles of secondary alkyl primary amine (Armeen L-9) having an average molecular weight of 170 and an average of 11 chain carbon atoms. The test results are given in Table II below.

TABLE II

| Run | Fuel          | Percent substituted urea | Viscosity increase, Percent | Fuel/air ratio | Fuel consumption, lbs./hr. | Percent decrease in fuel consumption | Hydrocarbon emission (NDIR) p.p.m. |
|-----|---------------|--------------------------|-----------------------------|----------------|----------------------------|--------------------------------------|------------------------------------|
| 11  | Base fuel     | 0.10                     | 96                          | 0.0943         | 2.275                      | 11.8                                 | 425                                |
| 12  | Additive fuel |                          |                             | 0.0813         | 2.01                       |                                      | 307                                |

tistokes or by about 29% by the addition of a viscosity modifier when tested in a standard 1961 automobile en-

Additive fuels containing 0.20 and 0.25 weight percent of the same substituted urea in the above engine

test gave comparable improvement in fuel consumption and substantially higher reduction in hydrocarbon emissions than the 28% reduction in Run 12 above.

Obviously many modifications and variations of the invention, as hereinafter set forth, may be made without departing from the spirit and scope thereof, and therefore, only such limitations should be imposed as are indicated in the appended claims.

I claim:

1. A method of operating a spark-ignited internal combustion engine which comprises burning in said engine a motor fuel comprising a hydrocarbon mixture boiling in the gasoline boiling range containing an oil-soluble substituted urea, having the formula:



in which R and R' are each alkyl radicals having from 1 to 18 carbon atoms and the sum of the carbon atoms in said R and R' radicals collectively is at least 12, in an amount effective to increase the viscosity of said motor fuel measured as kinematic viscosity in centistokes by at least 10 percent to 200 percent over the viscosity of said hydrocarbon mixture.

2. A method according to claim 1 in which the viscosity of said motor fuel is increased by an amount from about 40 to 100 percent.

3. A method according to claim 1 in which said motor fuel contains from about 0.005 to 0.5 weight percent of said substituted urea.

4. A method according to claim 1 in which said substituted urea is the reaction product of 1 mole of toluene diisocyanate and 2 moles of n-C<sub>9</sub> alkyl primary beta amine.

5. A method according to claim 1 in which said substituted urea is the reaction product of 1 mole of toluene diisocyanate and 2 moles of n-C<sub>11</sub> alkyl primary beta amine.

6. A method according to claim 1 in which said substituted urea is the reaction product of 1 mole of toluene diisocyanate and 2 moles of C<sub>10-14</sub> secondary alkyl primary amine.

7. A motor fuel composition comprising a hydrocarbon mixture boiling in the gasoline boiling range containing an oil-soluble substituted urea having the formula:



in which R and R' are each alkyl radicals having from 1 to 18 carbon atoms and the sum of the carbon atoms in said R and R' radicals collectively is at least 12, in an amount effective to increase the viscosity of said motor fuel, measured as kinematic viscosity in centistokes by at least 10 percent to 200 percent over the viscosity of said hydrocarbon mixture.

8. A composition according to claim 7 in which the viscosity of said motor fuel is increased by an amount from about 40 to 100 percent.

9. A composition according to claim 7 in which said motor fuel contains from about 0.005 to 0.5 weight percent of said substituted urea.

10. A composition according to claim 7 in which said substituted urea is the reaction product of one mole of toluene diisocyanate and 2 moles of n-C<sub>9</sub> alkyl primary beta amine.

11. A composition according to claim 7 in which said substituted urea is the reaction product of 1 mole of toluene diisocyanate and 2 moles of n-C<sub>11</sub> alkyl primary beta amine.

12. A composition according to claim 7 in which said substituted urea is the reaction product of 1 mole of toluene diisocyanate and 2 moles of C<sub>10-14</sub> secondary alkyl primary amine.

#### References Cited

##### UNITED STATES PATENTS

40 3,082,170 3/1963 McCarthy et al. \_\_\_\_ 252—51.5  
3,164,138 1/1965 Reuter et al. \_\_\_\_ 44—66 XR

DANIEL E. WYMAN, Primary Examiner.

45 W. J. SHINE, Assistant Examiner.